

1

3,216,955

### ELECTRICAL RESISTOR

Samuel Ruben, 52 Seacord Road, New Rochelle, N.Y.  
No Drawing. Filed Apr. 23, 1963, Ser. No. 274,904  
2 Claims. (Cl. 252—512)

This invention relates to a stable refractory electrically conductive element and specifically to an electrical resistor.

A general object of the invention is to provide a material suitable for use as an electrical resistor.

Other objects will be apparent from the disclosure.

In the past there has been a general recognition that molybdenum disilicide is a useful base material for electrical resistance elements. In my Patent 3,006,865 I have described a refractory composition suitable for use as an electrical resistance element, comprising the reaction product of molybdenum disilicide and vanadium pentoxide. In my pending U.S. patent application Serial No. 144,292, filed October 11, 1961, I describe an improvement upon the device covered by my aforementioned patent.

The present invention has to do with a new composition, which for certain applications such as for electrical resistors, is an improvement over my patent and the pending patent application.

I have found that the composition of molybdenum disilicide and elemental boron provides a superior resistance element.

The art discloses many combinations of molybdenum disilicide and bonding reacting agents such as the borides, silicates and oxides. The use of these materials affect the electrical conductivity of the molybdenum disilicide and the resultant products are in most cases unable to withstand thermal shock.

I have produced an improved electrical resistor element by mixing and grinding molybdenum disilicide granules with elemental boron and heating to a temperature in the order of 1100° C. to 1200° C. A metal-like dense material is obtained, capable of sustained applications at high temperature, such as 1200° C., having good electrical conductivity and a positive resistance temperature coefficient.

The percent of boron added to the molybdenum disilicide determines the density of the combination, its resistivity and temperature coefficient. The preferred range of boron is from 2% to 20%, the balance being molybdenum disilicide. The resistance material composition is prepared by ball milling the molybdenum disilicide and boron particles in a carbide lined mill for several hours. For a typical resistor element, I ball mill a mixture of 90% molybdenum disilicide and 10% boron. Rods .046" by 8.25", are pressed at 30 tons per square inch and have a pressed density of 3.75/cc. The grain size of the boron and molybdenum disilicide particles is 1.5 microns as measured with a Fisher sub-sieve sizer. After pressing, the rods are heated in a furnace for 30 minutes at 1100° C. When cool the rods are extremely hard and possess good tensile strength.

Rods made with 5% boron added to 95% molybdenum disilicide are of a conductive refractory nature and have a resistivity of .0034 ohm cm. at 1200° C.; rods made with 10% boron, balance molybdenum disilicide have a resistivity of .0041 ohm cm. at 1200° C., and .00168 ohm cm. at room temperature. Continuous operation in oxidizing atmospheres produces negligible change in resistivity, mechanical strength or appearance.

If desired, terminals may be applied to the rods by a  $\frac{1}{2}$ " nickel plating on each end. The plated ends may then be placed in a hollowed copper rod and the space between the rod and the hollow copper rod terminal filled with silver solder. This low resistance type contact

2

is useful in resistors which are continuously operated over long periods of time and serve to maintain a low contact resistance. The copper rod contacts may be of sufficient mass to dissipate enough energy to keep the ends cool.

5 The positive resistance temperature coefficient characteristic of the resistor of this invention is important and keeps the current from progressively increasing to a destructive degree such as occurs with most semiconductors. If desirable, the positive temperature coefficient may be reduced by the addition of tin oxide or other refractory conductive oxides possessing a negative resistance temperature coefficient.

10 The particle size of the component elements, boron and molybdenum disilicide, influences the preferred mixture range in terms of resistivity and mechanical properties at high temperature operation.

15 An important characteristic which I have observed is that when the boron and molybdenum disilicide are reacted and bonded together there is small dimensional change, in the order of 1% with the pressures presently utilized. This permits objects having mechanical strength at high temperature to be produced by powder metallurgy processes.

20 25 An examination of the structure of the reaction product indicates that the elemental boron combines with some of the molybdenum disilicide and also that a small amount of the boron oxidizes to boric oxide which combines with silicates formed during the heating period.

30 35 To insure maximum electrical stability and density of a resistor element, it is heated prior to initial use, by an electric current discharged through it at a temperature beyond that at which the materials had been reacted. For example, a unit reacted at 1200° C. is heated to a temperature of about 1500° C. by discharging a current therethrough for a short time. This tends to equalize the resistance over the length of the unit.

40 45 The resistivity of the composition may be increased by the addition of such refractory conductive materials as the nitrides, borides or carbides of Zr, Ti, Ta, Va or Cr; also by the addition of refractory non-conductors such as micronized aluminum oxide and the silicates and oxides of zirconium.

50 55 As the compositions of this invention lend themselves to pressing into the desired shape prior to reaction, it is possible to produce circular resistor elements for use in rheostats or potentiometers, in place of wire wound types which tend to oxidize under overload or when operated at maximum rated capacity.

I claim:

1. An electrical resistor element consisting essentially of 2% to 20% boron, the balance being substantially all molybdenum disilicide, said resistor element being the product of heating a pressed mixture of boron and molybdenum disilicide particles in the desired proportion to a temperature of about 1100° to 1200° C. for a time sufficient to cause reaction of said particles in the mixture.

2. An electrical resistor element as claimed in claim 1, which contains a small amount of boric oxide.

#### References Cited by the Examiner

#### UNITED STATES PATENTS

2,463,404 3/49 McKinley ----- 264—57  
2,745,928 5/56 Glaser ----- 252—518 XR

#### OTHER REFERENCES

Dummer: Fixed Resistors. Pitman & Sons (1956), page 92.

70 JULIUS GREENWALD, Primary Examiner.

ALBERT T. MEYERS, Examiner.